

## UNITED STATES PATENT OFFICE

2,102,502

## MAKING RIMMED STEEL

Rufus E. Zimmerman, Short Hills, N. J., and  
Clarence D. King, Brooklyn, N. Y.No Drawing. Application January 8, 1937,  
Serial No. 119,630

3 Claims. (Cl. 75—53)

Rimmed or effervescent steel is particularly valuable in steel products requiring ductility and the ingots of such steel are characterized chiefly by a skin which for a considerable depth, one to two inches, is uniform and dense and exceptionally clean or free from blow holes so that it rolls well.

The process of rimming is characterized by a boiling or an escape of gases during the solidification of the ingot in the mold, as distinguished from killed or partly killed steel which is quiescent in the mold.

For the best results the rimming or ebullition should be regular and fairly long continued, as distinguished from spasmodic escape of large bubbles of gas.

Rimming steels generally have been of low carbon content, below about .20 carbon (and in larger part below .10 carbon) and containing in the molten condition when tapped from the furnace a fairly high percentage of iron oxide (FeO); the evolution of the escaping gases being apparently caused by the generation of carbon monoxide in the molten metal.

In the very low carbon steels (.05 carbon and under) there normally exists sufficient iron oxide to assure maximum reaction with carbon when pouring the heat, and maximum rimming action, permitting the gases in the steel to escape freely and assuring proper thickness of good skin and location of blow holes. It is more difficult to produce constantly a properly rimmed ingot, that is, one with desired skin thickness and location of blow holes, with comparatively high carbon steels, say from .20 to .35 percent carbon.

Steels with comparatively low iron oxide content are also more difficult to rim properly, as are those of high manganese content and those tapped at high temperatures; and comparatively large ingots present a special difficulty because the rimming action is not as pronounced as in the casting of small ingots. With these compositions and these conditions thin skinned ingots often result with blow holes close to the surface. Frequently such blow holes are exposed on heating in soaking pits prior to rolling, resulting in defects in the steel when rolled. They are also objectionable in the finished product because of their close proximity to the surfaces of the steel.

We have discovered that the rimming operation can be improved and the quality of the rimmed steel bettered by the addition of a borate such as borax or boric-acid or a borax glass or other boron-oxygen compounds after tapping

and that such agents are particularly effective in the more difficult steels referred to above containing .20 per cent or more carbon and having an unusually low iron oxide content. Commercial borax may be used having the formula  $Na_2B_4O_7 \cdot 10H_2O$ . It should be dehydrated to remove all or most of the 10 molecules of water of crystallization by heating to 500 degrees C. or higher, as by roasting, fusing or sintering or the like. Or borax glass may be used, or a mixture of ordinary glass, comprising sodium and calcium silicates, with boric acid or borax, may be used. The quantity used may be varied from one ounce to one pound of borax per ton of steel. It may be added, wholly or in part, in the ladle but is preferably introduced into the ingot mold while pouring, shortly after beginning the teeming operation.

For example, we have found that the addition of dehydrated commercial borax to the extent of two or three ounces per ton of ingot results in good rimming action in steels which inherently lack this characteristic, such as steels containing .20 carbon and higher, with a decided improvement in the rolling characteristics of the product, better surface, less rejections of material and less chipping or reconditioning of the partially rolled steel, and less scrap.

In the rimming operation there is normally a drop in the top level of the ingot during the early stages of solidification. There is generally a rise of the top level as the steel freezes; the better the rimming action, the smaller the rise.

Taking steels which are generally recognized as most difficult to rim, running from .23 to .30 carbon and adding borax from about one and one-quarter ounces to three ounces per ton of ingot, we have secured a good rimming action with a growth of the ingot at the end of less than three inches and in nearly all cases less than two inches, which is good rimming practice. Photomicrographs of sections of the blooms, billets and bars rolled from these ingots showed that the blow holes had been favorably seated, that is, in the middle portion of the rolled products, with the desired pattern of the skin or case and the core such as are found in good rimmed steel.

The quantity of the boric-acid-containing or borax-containing agent may be varied and can be readily adjusted to the most economical point to produce the best rimming ingot in accordance with the conditions referred to above. In adding the agent to the molds the commonly preferred practice is to introduce it near the bot-

tom immediately after starting a full pouring stream of metal.

Similar treatment of steels with less than .20 carbon showed good results, although the chief importance of the invention is apparently in its providing a good rimming action where it has previously been difficult to secure this.

Various modifications may be made by those skilled in the art without departing from the invention as defined in the following claims.

What we claim is:

1. The method of making rimmed steel ingots which comprises the addition of about two to three ounces of dehydrated borax per ton of

metal to the molten steel while pouring the ingot.

2. The method of rimming steel containing carbon over .20 per cent which comprises the addition to the molten steel after tapping of a small percentage (of the order of a few ounces per ton of steel) of a member of the group consisting of boric-acid and the borates. 5

3. The method of rimming steel containing carbon over .20 per cent which comprises the addition to the molten steel while pouring the 10 ingot of about 2 or 3 ounces of dehydrated borax per ton of steel.

RUFUS E. ZIMMERMAN.  
CLARENCE D. KING.